

(No Model.)

S. HEIMANN.

ELECTRODE FOR ELECTRIC ARC LAMPS.

No. 498,915.

Patented June 6, 1893.



WITNESSES:

*Charles Schroeder.*  
*Harry Willard Griffiths.*

INVENTOR

*S. Heimann*  
BY *Guyot & Baumann*

ATTORNEYS.

# UNITED STATES PATENT OFFICE.

SALOMON HEIMANN, OF NEW YORK, N. Y.

## ELECTRODE FOR ELECTRIC-ARC LAMPS.

SPECIFICATION forming part of Letters Patent No. 498,915, dated June 6, 1893.

Application filed October 24, 1892. Serial No. 449,775. (No model.)

*To all whom it may concern:*

Be it known that I, SALOMON HEIMANN, a citizen of Germany, residing in the city of New York, in the county of New York and State of New York, have invented certain new and useful Improvements in Electrodes for Electric-Arc Lamps, of which the following is a specification.

The object of my invention is to treat carbons for electric arc lamps in such a manner as to prevent the rapid consumption of the carbons by the light arc and the influence of the atmosphere; and the invention consists in a carbon provided with a coating of a mixture of powdered calcined soapstone, water-glass and oil and lamp-black in proportions that will be set forth hereinafter.

In the accompanying drawing, a longitudinal sectional view of my improved carbon is shown.

The carbon A, which may have any desired dimensions, is provided with a coating *a* of refractory material, which coating has a thickness of about one sixty-fourth to one thirty-second of an inch, so as not to interfere with the easy movement of the carbon in passing through apertures in guard-plates, reflectors, &c. This coating is preferably made of the following mixture: seventy parts by weight of powdered calcined soapstone, five parts by weight of water-glass, twenty parts by weight of oil and five parts of lamp black. These materials are thoroughly ground together and mixed with enough water to give them about the consistency of cream. The carbon is then dipped into the same until a coating adheres

to the same of from about one sixty-fourth to one thirty-second of an inch in thickness, and then the carbon is dried for one or two days. This coating is refractory and protects the carbon from the influences of the atmosphere and the light arc, except at the point of the arc.

I am aware that carbons in electric lamps have been provided with a coating of plaster of paris, for example, the well known Jabllochhoff candle, and that carbons and filaments have been coated with enamel, glass, clay, &c., but these differ totally from my improved carbon, as the coating of my improved carbon is very thin and can crumble away at the point of the arc as the carbon is consumed, and thus prevents the formation of craters, and protuberances which are so very objectionable in arc lamps; but at the same time this improved coating fully protects the carbon from the influence of the atmosphere and the electric light arc.

Having thus described my invention, I claim as new, and desire to secure by Letters Patent—

An electric arc light carbon, provided with a refractory coating composed of a mixture of calcined soapstone, water-glass, oil and lamp-black about in the proportions given.

In testimony that I claim the foregoing as my invention I have signed my name in presence of two subscribing witnesses.

SALOMON HEIMANN.

Witnesses:

OSCAR F. GUNZ,  
CHARLES SCHROEDER.